

## UNITED STATES PATENT OFFICE

2,487,569

ANTISTAIN BATHS FOR COLOR  
PHOTOGRAPHIC MATERIALSE. Scudder Mackey, Binghamton, N. Y., assignor  
to General Aniline & Film Corporation, New York,  
N. Y., a corporation of DelawareNo Drawing. Application July 21, 1948,  
Serial No. 40,010

4 Claims. (Cl. 95—88)

1

This invention relates to photographic anti-stain baths, to anti-stain baths employed in multi-layer color photography, and especially to final rinse baths for the washing of multi-layer color photographic material following the fixing treatment so as to prevent the formation of stain.

It is known that in the processing of multi-color reversible film and multi-color reversible white opaque the exposed film or exposed white opaque, is first developed with a normal black and white developer to produce a negative image. After development, the black and white negative material, without being fixed, is exposed to general illumination, followed by a second development with a color-forming developer. During the first and second development, the silver-halides in all the layers are reduced to metallic silver. After the second development, the material is cleared in running water, hardened in an aqueous solution consisting of either alum or potassium chrome alum, and then washed in running water. After the latter treatment, the silver present in all the layers formed during the first and second development is converted into a salt by any of the known silver-salt formers, commonly known as bleaching baths, and the silver-salt thus formed is then removed by dissolving it in a silver-salt solvent such as, for example, hypo. The material is then washed for a long period of time and then dried.

During the final washing operation it is essential that the residual second or color developer and bleach solutions be removed, otherwise stains will be formed during the drying operation, which are particularly noticeable in the white area. In order to prevent this staining, an extended final washing time in running water of from fifteen minutes to two hours has been proposed. Even if this proposal be adopted, stains are nevertheless formed during and after the drying operation. It is believed that the staining results from the oxidation of traces of the color developer retained in the layers of the material following color-forming development, which then react with the unused color former.

An object of the present invention is to eliminate excessive washing time of color developed multi-color photographic material while preventing the formation of stain.

A further object of the invention is a final rinse bath which clears undesirable matter from a multi-color photographic material in a short time while avoiding staining.

Other objects and features of the invention will become apparent as the description proceeds.

I have discovered that the above objects are accomplished by employing as a final rinse bath an aqueous solution containing a small quantity of a water-soluble addition product of formaldehyde and a diazine or triazine. The diazines and

2

triazines contemplated for reaction with the formaldehyde have the following formulae:

(1)



(2)



and

(3)



In Formula 1 at least one Y is an amino group having at least one reactive hydrogen atom, the remaining Y's being a radical such as hydrogen, amino, hydroxy, halogen, i. e., chlorine, bromine, etc., alkyl, i. e., methyl, ethyl, propyl, isopropyl, butyl, etc., alkylene, i. e., 1-buteneyl, etc., aryl, i. e., phenyl, naphthyl, etc., and aralkyl, i. e., benzyl, methylbenzyl, ethylbenzyl, etc. In Formula 2 Z represents hydrogen, amino, alkyl, i. e., methyl, ethyl, butyl, etc., phenyl, phenylene, hydroxy, alkoxyl, i. e., methoxy, ethoxy, propoxy, etc., mercapto, alkylthio (alkyl-S-), i. e., methylthio, ethylthio, propylthio, etc., and hydrazino, at least two Z's being primary amino or hydrazino. In Formula 3 X is hydrogen or a primary amino and R represents halogen, hydrazino, phenyl, hydroxy, alkoxy, i. e., methoxy, ethoxy, propoxy, butoxy, etc., or an alkylthio (alkyl-S-) group, i. e., methylthio, ethylthio, propylthio, etc.

The water-soluble addition products of formaldehyde and an azine characterized by Formula 1 are prepared according to the methods described in United States Patent 2,197,357. The water-soluble products while utilizing the azines of Formulae 2 and 3 are prepared according to the methods described in United States Patents, 2,211,710 and 2,211,709, respectively.

By utilizing this final rinse bath, in lieu of extended washing in water, the washing time after fixing is considerably reduced, and stain formation prevented. The exact operation of the water-soluble addition products of formaldehyde and an azine in the final rinse bath is unknown and to date has been unascertainable. It is known that the tendency to stain formation encountered in the processing of color film by the color forming development method is attributable

in the main to the retention in the layers of the multi-layer material of small amount of the color developer. This becomes progressively oxidized by atmospheric conditions, the oxidized products reacting with unused and unremoved color former.

It is likewise known that this tendency to stain formation can be obviated by the utilization of reducing agents such as alkali sulfite, hydrazines, hydroxylamines and the like which operate to destroy the retained color developer. Rather peculiarly, it has been found that the addition products referred to hereinabove are analogous to the reducing agents to the extent that both overcome the tendency to stain formation. Despite the fact that the addition products would not appear to be constituted in a fashion to permit them to act as reducing agents, it would, nevertheless, appear that they may have this property because of the results they achieve. In any case, the conclusion is inescapable that the addition products either function as reducing agents to destroy the color developer, or react with the color developer or the oxidation products thereof in a manner to prevent subsequent reaction of the color developer with retained color former.

The concentration of the addition products required may vary from as little as 0.5%, an amount which in general has been found to eliminate stain for the most part, to as much as 5%, an amount which is an assurance that stain formation will not ensue. Amounts higher than 5% give little improvement. Concentrations ranging from between 2 and 4% are most desirable from a commercial standpoint.

The photographic multi-layer materials, which may be processed with the anti-stain bath of the present invention, are color reversible film, color negative film, color reversible white printing material coated on an opaque base, and color positive printing material coated on paper, irrespective of whether the dyestuff images are produced with color formers present in the emulsion, or by a selective second exposure followed by development with developing solutions containing color formers and color developing agents.

The color reversible film consists of an integral tripack emulsion coated on the usual clear cellulose acetate or nitrate film base. Each of the emulsion are sensitized to one of the primary colors of light, namely, blue, green, and red. The top layer is blue sensitive. A filter layer, yellow in color and blue absorbing, lies under the top layer. Below this filter layer, lies a green sensitive emulsion layer, and below this is a red sensitive emulsion layer. Each of the three silver-halide emulsion layers contain dye-forming compounds which unite during the development of a silver image in an aromatic amine developing agent to form a dye with the oxidation product of the developing agent, or may be free from color formers in which case the film is processed with the color formers in the color developers by the selective second exposure and color development method as described in United States Patents 1,897,866, 1,900,870, 1,928,709 and 1,980,941.

As silver is formed during development, it must be removed after color development by treatment in a bleach, followed by treatment in a bath of sodium thiosulfate, according to usual practice. A yellow dye is formed in the blue sensitive emulsion; a magenta dye is formed in the green sensitive emulsion; and a cyan dye is formed in the red sensitive emulsion. Combinations of these

three printing primaries will produce all of the other colors in the finished film or print.

The color negative film is made up in the same manner as the color reversible film with the exception that it may contain a layer of clear gelatin between the red sensitive layer and the green sensitive layer. The color reversible white opaque material is prepared in the same manner as color reversible film and the color negative film with the exception that the base consists of an opaque white film. The color paper is also constructed in the same manner as the color reversible film and the color negative film, with the exception that the emulsion is coated on a baryta coated paper base. Suitable methods for the preparation of photographic multi-layer materials have been described in the literature relating to color photography and are, therefore, not described here.

The following examples describe in detail methods for accomplishing the above objects, but it is to be understood that they are inserted merely for purposes of illustration and are not to be construed as limiting the scope of the invention.

#### Example I

A 4" x 5" full color transparency sheet of color film was printed by contact on two 4" x 5" sheets of color reversible white opaque film.

The two sheets of 4" x 5" color reversible white opaque film were first developed for twelve minutes at 68° F. in a developer of the following composition:

|                                 |       |    |
|---------------------------------|-------|----|
| p-Monomethylaminephenol sulfate | grams | 3  |
| Sodium sulfite                  | do    | 50 |
| Hydroquinone                    | do    | 6  |
| Sodium carbonate (monohydrate)  | do    | 40 |
| Sodium thiocyanate              | do    | 2  |
| Potassium bromide               | do    | 2  |
| Water to make                   | liter | 1  |

The developed film was short stopped for three minutes at 68° F. in a 5% aqueous solution of sodium bisulfite.

The film was washed for two minutes in running water 68° F. and re-exposed to white light.

The re-exposed film was color developed for fifteen minutes at 68° F. in a developer of the following composition:

|                           |       |    |
|---------------------------|-------|----|
| p-Aminodiethylaniline HCl | grams | 4  |
| Sodium sulfite            | do    | 20 |
| Hydroxylamine HCl         | do    | 2  |
| Sodium carbonate          | do    | 80 |
| Potassium bromide         | do    | 1  |
| Water to make             | liter | 1  |

The color developed film was rinsed for four minutes in running water at 68° F., and hardened for five minutes in a 3% aqueous solution of potassium chrome alum.

The hardened film was washed for five minutes in running water at 68° F. The washed material was then treated with a bleach bath of the following composition:

|                                        |                   |     |
|----------------------------------------|-------------------|-----|
| Di-potassium mono-sodium ferri-cyanide | grams             | 100 |
| Potassium bromide                      | do                | 15  |
| Disodium phosphate                     | do                | 40  |
| Sodium bisulfate                       | do                | 25  |
| Formalin (40%)                         | cubic centimeters | 20  |
| Water to make                          | liter             | 1   |

The bleached film was washed for five min-

## 5

utes at 68° F., and then fixed for five minutes in a solution of the following composition:

|               |       |     |
|---------------|-------|-----|
| Hypo          | grams | 200 |
| do            | do    | 10  |
| Borax         | liter | 1   |
| Water to make |       |     |

After fixing, the material was washed for ten minutes in running water at 68° F.

After the final washing, one print was allowed to dry while the other was rinsed for five minutes in an aqueous solution consisting of 98 parts by weight of water and 2 parts by weight of a water-soluble addition product of formaldehyde and cyanurtrihydrazide, methylol-cyanurtrihydrazide, prepared according to Example I of United States Patent 2,211,709, and then allowed to dry. At this point, the prints appeared identical. After normal drying, the print rinsed in the solution containing the addition product of formaldehyde and cyanurtrihydrazide showed brighter colors and more brilliant highlights. The print given only a water washing for five to twenty minutes showed a slight highlight stain.

When the drying was carried out under conditions of high humidity so that the drying time was extended for several hours, the water-rinsed print showed even greater highlight stains while the print rinsed in the aqueous solution containing the addition product did not change.

After storing both prints, i. e., treated and untreated for several months, it was observed that the color balance of the treated print was unaffected, whereas the color balance of the untreated print was completely ruined by yellow stain appearing overall, while at the same time the densities of the original yellow image were lowered.

## Example II

Example I was repeated with the exception that the colored material employed was a color paper and the final rinse bath consisted of 98 parts by weight of water and 2 parts by weight of a water-soluble addition product of formaldehyde and 2,4,6-triaminopyrimidine, 2,4,6-trimethylolaminopyrimidine, prepared according to Example I of United States Patent 2,211,710. The color print washed in water showed objectionable stains on slow drying, while the print washed with the aqueous solution containing the addition product was clear and unstained.

## Example III

Example I was repeated with the exception that the colored material employed was a color transparency sheet and the final rinse bath consisted of 97 parts by weight of water and 3 parts by weight of a water-soluble addition product of formaldehyde and melamine, trimethylolmelamine, prepared according to Example VI of United States Patent 2,197,357. After fixing and washing, the color print washed in water showed objectionable stains, while the color print treated with the aqueous solution containing the addition product was clear and unstained.

## Example IV

Example I was repeated with the exception that the final rinse consisted of 98 parts by weight of water and 2 parts by weight of trimethylolmelamine available commercially under

75 wherein at least one Y is an amino group having

## 6

the brand name of Tanak MRX and having the following formula:



The color print washed in water showed objectionable stains after drying, while the print treated with the solution containing the trimethylolmelamine was clear and unstained.

Similar results were obtained as in the preceding examples when the addition products of Examples 2, 4, and 5 of United States Patent 2,211,709, Examples 3, 4, and 16 of United States Patent 2,211,710, and Examples 4, 7, and 15 of United States Patent 2,197,357 were employed.

The treated and untreated prints of Examples II to IV inclusive were stored for several months. The untreated prints showed marked staining during storage and the color balance after storage was completely ruined by yellow stains, whereas no stains were evident on the treated prints and the color balance was unaffected.

Instead of employing the water-soluble addition products of formaldehyde and an azine in aqueous solutions as a final rinse bath, they may be incorporated into gelatin solutions in a concentration ranging from 2-5% and such gelatin solutions utilized as a surface coating for the processed multi-layer photographic material.

The above specific examples are to be regarded as being merely illustrative of the invention and not in any sense restrictive. It will be obvious to those skilled in the art that many modifications, such as substituting equivalent materials and varying the proportions of the materials used, may be made. The scope of the invention is to be limited solely by the appended claims.

I claim:

1. In a process of producing color photographic images in a silver-halide emulsion by exposing the emulsion, color-forming developing the same, bleaching, fixing, and washing, the improvement which comprises avoiding the formation of stain, after the bleaching and washing operation, by rinsing the said silver-halide emulsion with an aqueous solution containing a water-soluble addition product of formaldehyde and an azine selected from the class consisting of those having the following formulae:



and



at least one reactive hydrogen atom, the remaining Y's being a radical selected from the group consisting of hydrogen, hydroxyl, halogen, alkyl, alkylene, aryl and aralkyl, Z represents a member selected from the group consisting of hydrogen amino, hydroxy, alkyl, alkoxy, phenyl, phenylene, mercapto, alkylthio and hydrazino, at least two Z's being a member selected from the class consisting of amino and hydrazino group, X represents a member selected from the group consisting of hydrogen and a primary amino group, R represents a member of the group consisting of halogen, hydroxy, hydrazino, alkoxy, phenyl, and alkylthio groups.

2. In a process of producing color photographic images in a silver-halide emulsion by exposing the emulsion, color-forming developing the same, bleaching, fixing, and washing, the improvement which comprises avoiding the formation of stain, after the bleaching and washing operation, by rinsing the said silver-halide emulsion with an aqueous solution containing methylolcyanurtrihydrazide.

3. In a process of producing color photographic images in a silver-halide emulsion by exposing the emulsion, color-forming developing the same,

bleaching, fixing, and washing, the improvement which comprises avoiding the formation of stain, after the bleaching and washing operation, by rinsing the said silver-halide emulsion with an aqueous solution containing 2,4,6-trimethylolaminopyrimidine.

4. In a process of producing color photographic images in a silver-halide emulsion by exposing the emulsion, color-forming developing the same, bleaching, fixing, and washing, the improvement which comprises avoiding the formation of stain, after the bleaching and washing operation, by rinsing the said silver-halide emulsion with an aqueous solution containing trimethylolmelamine.

E. SCUDDER MACKEY.

#### REFERENCES CITED

The following references are of record in the file of this patent:

#### UNITED STATES PATENTS

| Number    | Name     | Date           |
|-----------|----------|----------------|
| 2,384,658 | Vittum   | Sept. 11, 1945 |
| 2,440,954 | Jennings | May 4, 1948    |